

# United States Patent

[19]

Joy et al.

[11] 3,855,326

[45] Dec. 17, 1974

[54] **PRODUCTION OF OLEFINIC HYDROCARBONS**

[75] Inventors: **David Richard Joy; Pannalal Sohanlal Jhawar**, both of Stockton-on-Tees, England

[73] Assignee: **Imperial Chemical Industries Limited**, London, England

[22] Filed: **Nov. 29, 1973**

[21] Appl. No.: **420,092**

**Related U.S. Application Data**

[63] Continuation-in-part of Ser. No. 136,547, April 22, 1971, abandoned.

[30] **Foreign Application Priority Data**

May 8, 1970 Great Britain ..... 22348/70

[52] U.S. Cl. ..... 260/666 PY

[51] Int. Cl. ..... C07c 5/24

[58] Field of Search ..... 260/666 PY

[56] **References Cited**

UNITED STATES PATENTS

2,704,778 3/1955 Maisel ..... 260/681.5 R

2,752,406 6/1956 Seyfried ..... 260/666 PY

3,427,360 2/1969 Makowski ..... 260/666 PY

3,763,253 10/1973 Wing et al. ..... 260/666 PY

3,766,283 10/1973 Lorette ..... 260/666 PY

Primary Examiner—Delbert E. Gantz

Assistant Examiner—Veronica O'Keefe

Attorney, Agent, or Firm—Cushman, Darby & Cushman

[57] **ABSTRACT**

A mixture of olefinic hydrocarbons useful as a termonomer in EPDM rubbers contains 2-propen-1-yl-norbornene-5 and is produced by distilling a pyrolysis gasoline fraction to produce a distillate boiling in the range 10° to 80°C and separating this distillate fraction by redistillation into an isoprene-containing fraction and a piperylene-containing fraction. The piperylene fraction is heat-soaked at a temperature in excess of 150°C to produce the desired olefinic mixture. As an alternative feature of the process a part or all of the cyclopentadiene in the pyrolysis gasoline may be removed by heat-soaking at 100°-120°C, cyclopentadiene being re-introduced at a later stage in the process to produce a preferred mole ratio of 0.5 to 3 : 1 in the piperylene fraction before the latter in turn is heat-soaked.

15 Claims, No Drawings

## PRODUCTION OF OLEFINIC HYDROCARBONS

This is a Continuation-in-Part of our copending U.S. application Ser. No. 136,547 filed Apr. 22, 1971 and now abandoned.

The present invention relates to the production of mixtures of olefinic hydrocarbons, particularly mixtures of olefinic hydrocarbons suitable for copolymerisation with ethylene and propylene.

Co-polymers of ethylene and propylene with a third co-monomer are known to be products possessing valuable elastomeric properties and are frequently referred to as EPDM rubbers. The third monomer is generally a molecule containing at least two olefinic bonds, one of which takes part in the polymerisation process with the ethylene and propylene while the other remains unreacted and is, therefore, available for a subsequent vulcanisation process in which cross-linking takes place between polymer chains.

A wide variety of compounds have been suggested as the third co-monomer among which may be instanced 5-ethylidene norbornene-2, 1,4-hexadiene and dicyclopentadiene. The majority of these third co-monomers are derived from olefines which are themselves of petroleum origin and either the olefines or co-monomer or both are the subject of complicated and expensive extraction processes to obtain them in suitably pure form.

The cost of the third co-monomer is an appreciable factor in the cost of the finished co-polymer, not necessarily because of a high level of incorporation, but because of its cost of production. We have now devised a process in which a relatively crude unrefined hydrocarbon mixture may be used to produce a mixture of di-olefines which on polymerisation with ethylene and propylene produce a co-polymer with properties as good as those of a co-polymer produced from ethylene and propylene and one of the more conventional substantially pure co-monomers.

According to the invention a process for the production of a mixture of olefinic hydrocarbons suitable for co-polymerisation with ethylene and propylene comprises:

- a. distilling a pyrolysis gasoline fraction derived from a cracked hydrocarbon feedstock to produce a distillate boiling in the range 10° to 80°C and comprising piperylene and isoprene,
- b. re-distilling said distillate to produce an "isoprene concentrate" and a "piperylene concentrate," and
- c. heating said "piperylene concentrate" at a temperature of at least 150°C.

A pyrolysis gasoline fraction is obtained when a hydrocarbon feedstock is cracked with the aim of producing ethylene and propylene by heating to an elevated temperature, e.g. in the range 700° to 900°C and the cracked product distilled. The distillation may be carried out continuously in a series of distillation columns and the pyrolysis gasoline is obtained as a distillate fraction. The pyrolysis gasoline usually boils in the approximate range 0° to 200°C and consists of a number of saturated and unsaturated aliphatic hydrocarbons, naphthenes and aromatic hydrocarbons containing 4 to 10 carbon atoms. Notable constituents of the pyrolysis gasoline fraction are isoprene, piperylene, cyclopentadiene, pentanes, pentenes, hexanes, hexenes, cyclopentane, cyclopentene, styrene, cyclohexane, methylcyclo-

hexane, benzene, toluene and xylenes. The hydrocarbon feedstock which is employed in the cracking process is generally of petroleum origin and may be one of the crude oil distillation fractions, such as naphtha (boiling range 32° to 205°C), kerosine (boiling range 205°C to 260°C) or light or heavy gas oil (boiling ranges 205° to 315°C and 315° to 430°C respectively). Steam is generally added during the cracking process and a steam cracked naphtha is a preferred source of the pyrolysis gasoline for use in the present process.

Before it is used as feedstock in the process of the present invention, the pyrolysis gasoline is generally first subjected to a distillation in which C<sub>4</sub> hydrocarbons such as butadiene and butenes are removed as an overhead fraction. The residue from this distillation is then suitable for use in stage (a) of the process of the present invention to produce a distillate boiling in the range 10° to 80°C. The residue from this stage (a) distillation which comprises aromatic hydrocarbons, naphthenes and higher boiling olefines and paraffins may be submitted to separation processes, e.g. distillation and/or solvent extraction processes to produce aromatics, such as benzene and toluene and naphthenes such as cyclohexane.

The distillate fraction boiling in the range 10° to 80°C, preferably boils in the range 20° to 60°C and comprises piperylene and isoprene. It may also contain cyclopentadiene, n-pentane, isopentane, pentene-1, trans-pentene-2, 2-methylbutene-2, cyclopentene and cyclopentane.

The cyclopentadiene may be present as its dimer, di-cyclopentadiene and the piperylene may be present in one or both of its cis and trans forms.

If desired the cyclopentadiene and its dimer may be removed wholly or in part in an additional step immediately before or immediately after the distillate fraction is split into isoprene and piperylene concentrates. This may be achieved by heating the distillate fraction or the "piperylene concentrate" in a sealed system to a temperature of 100° to 120°C, preferably for ½ - 5 hrs., particularly 1 - 2 hrs. for partial conversion, or 3 - 4 hrs. for total conversion of cyclopentadiene to dicyclopentadiene. The latter is separated from the distillate fraction or the piperylene concentrate by distillation when the piperylene and other components are taken off as a distillate and the dicyclopentadiene remains as the residue.

The fraction boiling in the range of 10° to 80°C is divided by distillation into an "isoprene concentrate" (the distillate) suitably boiling in the range 10° to 40°C and a "piperylene concentrate" (the residue). The isoprene fraction may contain other lower boiling components, e.g. isopentane, n-pentane, and pentene-1 and may be suitably further refined, e.g. by distillation to recover substantially pure isoprene. The "piperylene concentrate" may contain higher boiling compounds such as cyclopentadiene/dicyclopentadiene, n-pentane, trans-pentene-2, 2-methylbutene-2, cyclopentene, cyclopentane and a trace of benzene. If desired this "concentrate" may be subjected to a distillation to remove one or more of the components boiling higher and/or lower than piperylene before undergoing the reaction stage (c) (for example, the removal of cyclopentadiene as described above). All of the foregoing distillations are preferably carried out continuously in a series of distillation columns in which the residue or distillate from one column forms the feed to the next.

The piperylene concentrate is heated at a temperature of at least 150°C, preferably 150° to 350°C, more preferably 150° to 250°C, for periods of up to 24 hours, e.g. 0.01 hrs. or more such as 1 to 24 hrs. Typically, heating periods will vary between 8 hours at 170°C to 15 minutes at 220°C. The intention of this heating step is to cause the cyclopentadiene and the piperylene in the piperylene concentrate to co-dimerise so if necessary cyclopentadiene and/or piperylene may be added before stage (c) to produce the ratio of cyclopentadiene to piperylene required. Addition of cyclopentadiene is especially necessary if the cyclopentadiene originally present in the fraction boiling in the range 10° to 80°C has been removed before or after division of the latter into the "isoprene concentrate" and "piperylene concentrate." The cyclopentadiene may be present or may be added in the form of its dimer which dissociates to cyclopentadiene during the reaction. It is preferred that the mole ratio of cyclopentadiene to piperylene in the piperylene concentrate be in the range 0.5 to 3 : 1, more preferably 0.5 to 1.2 : 1, especially 0.5 to 0.7 : 1. The piperylene concentrate with or without added cyclopentadiene is preferably heated in a sealed system under its autogenous pressure at the relevant temperature. The cyclopentadiene and piperylene co-dimerise to produce one or more of 4-methyl-4,7,8,9-tetrahydroindene, 7-methyl-4,7,8,9-tetrahydroindene, 2-vinyl-3-methyl norbornene-5 or 2-propen-1-yl-norbornene-5, desirably the latter. In addition both the piperylene and the cyclopentadiene may dimerise to give a number of isomeric decadienes and dicyclopentadiene respectively. The product of the process, therefore, may contain one or more of the dimers described as well as unreacted components originally present in the piperylene concentrate. It is usually preferable to remove these unreacted components, e.g. by distillation, to leave the mixture of dimers which are suitable for incorporation in a polymer without further treatment. If desired, however, one or more of the dimers may be separated from the product mixture and used individually or together in a polymer preparation. For example, it is preferred that a fraction be distilled from the product of the process boiling in the range 80° to 87°C at 50 mm. Hg and comprising at least 50 percent, preferably at least 90 percent, by weight 2-propen-1-yl-norbornene-5. This fraction provides a very effective third monomer.

The invention will now be further described with reference to the following Examples.

#### EXAMPLE 1

A debutanised pyrolysis gasoline fraction boiling in the range 0° to 200°C and derived from a stream cracked naphtha was distilled to produce a fraction of boiling range 10° to 80°C. This fraction was redistilled in a 30 tray Oldersaw batch distillation column under atmospheric pressure and a distillate taken boiling in the range 20° to 37°C comprising isoprene, n-pentane, iso-pentane and pentene-1 (isoprene concentrate). The residue from this distillation (piperylene concentrate) comprised 34 wt. percent cyclopentadiene and dicyclopentadiene, 20 wt. percent trans-piperylene and 13 wt. percent cis-piperylene. Also present were n-pentane (11.15 wt. percent) trans-pentene-2 (1.72 wt. percent), 2-methyl-butene-2 (4.8 wt. percent), cyclopentene (7.04 wt. percent) cyclopentane (10.46 wt. percent) and benzene (5.13 wt. percent).

500 grams of the "piperylene concentrate" were heated in a stainless steel autoclave at 180° to 190°C under autogenous pressure (approximately 300 p.s.i.) for periods of 1 to 3 hours. After removal of undimerised material the product was suitable for copolymerisation with ethylene and propylene.

#### EXAMPLE 2

Example 1 was repeated to produce a "piperylene 10 concentrate" containing 30 wt. percent cyclopentadiene and dicyclopentadiene, 19 wt. percent trans-piperylene and 13 wt. percent cis-piperylene. The balance of the concentration was made up of the compounds described for the similar concentrate in Example 1. 3 Kilograms of the concentrate were heated in a stainless steel autoclave at 190°C for 3 hours. The product was then distilled and a fraction comprising 75 wt. percent 2-propen-1-yl-norbornene-5, 20 wt. percent dicyclopentadiene and 5 wt. percent piperylene dimers obtained.

20 The fraction was incorporated into a polymer as follows:

The polymerisation apparatus consisted of a flanged 25 flask provided with tubes for feeding and discharging gases, a stirrer, a thermometer and a serum cap through which the diene and catalyst could be introduced. The tube for introducing the gases reached the bottom of the vessel and the apparatus was kept at a constant temperature of -20°C.

30 The flask was filled half full with 684 parts of anhydrous heptane which was then saturated at -20°C by passing through it for 15 minutes a mixture of propylene and ethylene in a molar ratio of 4 : 1. The flow rate of the gas mixture was equivalent to 8.5 times the total volume of the solvent in the flask per minute. 1.9 parts of the mixture of dienes prepared as above was then introduced into apparatus followed by 0.302 part of diethyl aluminum chloride as a solution in about 0.52 part of heptane and 0.097 part of vanadium tetrachloride as a solution in about 1.0 part of heptane and polymerisation commenced immediately. After a polymerisation period of 15 minutes, 7.93 parts of methanol were added to deactivate the catalyst and the polymer solution was washed with dilute HCl to remove catalyst residues. The polymer was precipitated by addition of the solution to an excess of methanol. It was then spread out on a tray and dried overnight in a vacuum oven.

40 50 100 Parts by weight of the polymer were then compounded on a laboratory roll-mill with 1.5 parts of sulphur, 5 parts of zinc oxide, 1 part of stearic acid, 1.5 parts of tetramethylthiuram monosulphide, 0.5 part of mercaptobenzothiazole and 50 parts of HAF carbon black and a small sample of the thus compounded polymer was vulcanised in a Wallace-Shawburn Curometer. The Curometer indicated that a time of 9 minutes at 150°C was required to achieve 95 percent of the maximum cure.

55 60 65 Three separating samples of the remaining compounded polymer were cured in a hydraulic press at a temperature of 160°C for, respectively, 15, 20 and 30 minutes, to form  $\frac{1}{8}$  inch thick sheets.

60 65 Standard dumbbell-shaped specimens having between the shoulders a nick 1 inch long and  $\frac{1}{16}$  inch wide were cut from the cured sheets. The tensile strength at break, the modulus, and the elongation to break of each specimen were measured on a Type E tensometer

using a rate of elongation of  $20 \pm 2$  inches/minute at room temperature. The tensile strength was 178 kgm/sq.cm., the percent elongation to break 440 and the 300 percent modulus 135 kgm/sq.cm.

Under comparable conditions polymer prepared from ethylene, propylene and 1,4-endomethylene-6-methyl-1,4,5,8,9,10-hexahydronaphthalene (known to produce an excellent co-polymer with ethylene and propylene) gave the following results:

|                       |                     |
|-----------------------|---------------------|
| 95% cure time         | 15 minutes at 150°C |
| Tensile strength      | 173 kg/square cm.   |
| 300% modulus          | 112 kg/square cm.   |
| % elongation to break | 435                 |

### EXAMPLE 3

A "piperylene concentrate" was heated and distilled to produce a fraction comprising 55 wt. percent 2-propen-1-yl-norbornene-5, 9 wt. percent exo-dicyclopentadiene, 19 wt. percent endo-dicyclopentadiene, 8 wt. percent piperylene dimers, the balance being codimers of cyclopentadiene and piperylene not containing the propenylnorbornene structure.

This fraction was incorporated into a polymer in a similar manner to Example 2 using 2.8 parts of the mixture.

The polymer produced had the following properties:

|                  |                    |
|------------------|--------------------|
| 95% cure time    | 9 minutes at 160°C |
| Tensile strength | 185 kg/square cm.  |
| 300% modulus     | 165 kg/square cm.  |

We claim:

1. In a process for the production of a mixture of olefinic hydrocarbons suitable for copolymerisation with ethylene and propylene the following steps in combination,

- distilling a pyrolysis gasoline fraction derived from a cracked hydrocarbon feedstock to produce a distillate boiling in the range 10° to 80°C comprising piperylene, isoprene and at least one member of the group consisting of cyclopentadiene, dicyclopentadiene, n-pentane, isopentane, pentene-1, trans-pentene-2, 2-methylbutene-2, cyclopentene, cyclopentane and benzene,
- redistilling said distillate to produce an isoprene concentrate and a piperylene concentrate, the latter including piperylene and at least one hydrocarbon selected from the group consisting of cyclopentadiene, dicyclopentadiene, n-pentane, trans-pentene-2, 2-methylbutene-2, cyclopentene, cyclopentane and benzene,
- heating said piperylene concentrate at a temperature of at least 150°C for a period of time up to 24 hours with added cyclopentadiene or dicyclopentadiene if one or other of these latter is not present in sufficient amount so as to codimerise said piperylene and cyclopentadiene and produce a mixture of olefinic hydrocarbons including 2-propen-1-yl-norbornene-5, said mixture being suitable for polymerisation with ethylene and propylene.

2. The process of claim 1 in which the pyrolysis gasoline boils in the range 0° to 200°C and is derived from a steam cracked naphtha.

3. The process of claim 1 in which the distillate produced in stage (a) boils in the range 20° to 60°C.

4. The process of claim 1 in which cyclopentadiene and its dimer in the distillate obtained in step (a) are removed at least in part in an additional step before the distillate fraction from step (a) is split into isoprene and piperylene concentrates in stage (b).

5. The process of claim 1 in which the distillate fraction from stage (a) or the piperylene concentrate from stage (b) is heated in a sealed system at 100° to 120°C for ½ to 5 hours to convert any cyclopentadiene which is present to dicyclopentadiene which is then removed as the residue in a further distillation.

6. The process of claim 1 in which the piperylene concentrate is heated at a temperature in the range 150° to 250°C for a period up to 24 hours to produce 2-propen-1-yl-norbornene-5.

7. The process of claim 1 in which at least one member of the group consisting of cyclopentadiene and piperylene is added to the piperylene concentrate before stage (c) to provide the required ratio of cyclopentadiene and piperylene for said co-dimerisation.

8. The process of claim 1 in which the mole ratio of cyclopentadiene to piperylene in the piperylene concentrate is in the range 0.5 to 3 : 1.

9. The process of claim 1 in which the product of stage (c) is distilled to give a fraction boiling in the range 80° to 97°C at 5 mm. Hg and comprising at least 50 percent by weight 2-propen-1-yl-norbornene-5.

10. The process of claim 1 in which a steam cracked naphtha boiling in the range 0° to 200°C is

a. distilled to produce a distillate boiling in the range 10° to 80°C comprising piperylene and isoprene.

b. said distillate is redistilled to produce an isoprene concentrate boiling in the range 10° to 40°C and a piperylene concentrate boiling in the range 40° to 80°C,

(c) said piperylene concentrate is heated at a temperature in the range 150° to 250°C for a period of up to 24 hours, and

d. said heated piperylene concentrate is distilled to produce a fraction boiling in the range 80° to 87°C at 50 mm. Hg comprising at least 50 percent by weight 2-propen-1-yl-norbornene-5, said fraction being suitable for co-polymerisation with ethylene and propylene.

11. The process of claim 10 in which cyclopentadiene and its dimer are also present in the distillate of step (a) and these are removed wholly or in part in an additional step before the distillate fraction is split into isoprene and piperylene concentrates by heating said distillate fraction in a sealed system at 100° to 120°C for ½ to 5 hours to convert cyclopentadiene wholly or in part to dicyclopentadiene and removing said dicyclopentadiene as a residue in a distillation.

12. The process of claim 11 in which cyclopentadiene and/or piperylene are added to the piperylene concentrate after the redistilling in step (b) but prior to step (c) to produce a mole ratio of cyclopentadiene to piperylene in the range 0.5 to 1.2 : 1.

13. In a process for the production of a mixture of olefinic hydrocarbons suitable for copolymerisation with ethylene and propylene, the step which comprises heating a piperylene concentrate including piperylene and cyclopentadiene at a temperature in the range of at least 150°C for a period of time up to 24 hours to codimerise said cyclopentadiene and piperylene and pro-

duce a mixture of olefinic hydrocarbons including at least one member of the group consisting of 4-methyl-4,7,8,9-tetrahydroindene; 7-methyl-4,7,8,9-tetrahydroindene; 2-vinyl-3-methyl norbornene-5 and 2-propen-1-yl-norbornene-5, said mixture being suitable for polymerisation with ethylene and propylene, said piperylene concentrate being obtained by (a) distilling a pyrolysis gasoline fraction derived from a cracked hydrocarbon feedstock to produce a distillate boiling in the range 10° to 80°C comprising piperylene, isoprene and at least one member of the group consisting of cyclopentadiene, dicyclopentadiene, n-pentane, isopentane, pentene-1, trans-pentene-2, 2-methylbutene-2, cyclopentene, cyclopentane and benzene, and (b) redistilling said distillate to produce an isoprene concentrate and said piperylene concentrate, cyclopentadiene or dicyclopentadiene being added to said piperylene concentrate if not present in sufficient amount to codimerise with the piperylene.

14. In a process for the production of a mixture of olefinic hydrocarbons suitable for copolymerisation with ethylene and propylene, the following steps in combination,

- a. distilling a pyrolysis gasoline fraction derived from a cracked hydrocarbon feedstock to produce a distillate boiling in the range 10° to 80°C comprising piperylene; at least one member of the group consisting of cyclopentadiene and its dimer, and isoprene,
- b. redistilling said distillate to produce an isoprene concentrate and a piperylene concentrate, the latter including piperylene and cyclopentadiene,
- c. heating said piperylene concentrate at a tempera-

ture of at least 150°C for up to 24 hours to codimerise said cyclopentadiene and piperylene and produce a mixture of olefinic hydrocarbons including at least one member of the group consisting of 4-methyl-4,7,8,9-tetrahydroindene; 7-methyl-4,7,8,9-tetrahydroindene; 2-vinyl-3-methyl norbornene-5 and 2-propen-1-yl-norbornene-5, said mixture being suitable for polymerisation with ethylene and propylene.

15. In a process for the production of a mixture of olefinic hydrocarbons suitable for copolymerisation with ethylene and propylene, the following steps in combination,

- a. distilling a pyrolysis gasoline fraction derived from a cracked hydrocarbon feedstock to produce a distillate boiling in the range 10° to 80°C comprising piperylene, at least one member of the group consisting of cyclopentadiene and its dimer, and isoprene,
- b. redistilling said distillate to produce an isoprene concentrate and a piperylene concentrate, the latter including piperylene and cyclopentadiene,
- c. heating said piperylene concentrate at a temperature in the range 150° to 250°C for up to 24 hours to codimerise said cyclopentadiene and piperylene and produce a mixture of olefinic hydrocarbons including at least one member of the group consisting of 4-methyl-4,7,8,9-tetrahydroindene; 7-methyl-4,7,8,9-tetrahydroindene; 2-vinyl-3-methyl norbornene-5 and 2-propen-1-yl-norbornene-5, said mixture being suitable for polymerisation with ethylene and propylene.

\* \* \* \* \*